

No. 894,111.

PATENTED JULY 21, 1903.

J. H. BOYD.

SMELTING PROCESS.

APPLICATION FILED FEB. 24, 1903.



Witnesses

Otto E. Hoddick

Dena Nelson

Inventor

James H. Boyd

By W. H. D. [Signature]  
Attorney

# UNITED STATES PATENT OFFICE.

JAMES H. BOYD, OF DENVER, COLORADO.

## SMELTING PROCESS.

No. 894,111.

Specification of Letters Patent.

Patented July 21, 1908.

Application filed February 24, 1908. Serial No. 417,425.

To all whom it may concern:

Be it known that I, JAMES H. BOYD, a citizen of the United States, residing at the city and county of Denver and State of Colorado, have invented a certain new and useful Smelting Process; and I do declare the following to be a full, clear, and exact description of the invention, such as will enable others skilled in the art to which it appertains to make and use the same, reference being had to the accompanying drawings, and to the letters and figures of reference marked thereon, which form a part of this specification.

My invention relates to a new process of smelting ores without roasting. In my improved process the sulfur is removed from the ores below the fusion zones in the furnace by bringing it in contact with the carbon or coke of the fuel. The carbon unites with the sulfur forming a sulfid of carbon which is volatile and passes upward whereby it is burned or consumed in the smelting zone and converted into sulfurous acid.

At the present time two classes of smelting is practiced. One is known as the lead smelting process and the other the matte smelting process. In the former, ores are reduced or changed from sulfids to oxids by roasting which adds largely to the cost of treatment, as a large portion of the ores is sulfids; as depth is gained in the mines. After roasting and being properly mixed they are smelted with sufficient lead-bearing ores to collect the gold, silver and lead in the metallic state and the copper in a matte in connection therewith. The other or matte smelting is conducted without roasting and the gold, silver, lead and copper are reduced to a matte together and require further treatment for their separation. These processes are conducted in shaft furnaces known as water jacket furnaces.

In the first or lead smelting process there is a smelting zone where the ore is reduced to a liquid state and slag and copper matte drawn off at the bottom of the smelting zone, the lead, gold and silver passing to a lower zone or hearth altogether. The fusion zone or where ores are reduced to a liquid state extends only as far as the effective force of the blast extends, varying some as the pressure of the blast varies, but rarely exceeds twelve inches below the twy whole.

By the use of my process, all kinds of ores are smelted without roasting. If properly

mixed, the sulfids will reduce the oxids and all become sulfids, being thus reduced to a matte and slag in the fusion zone or space where the blast enters. This matte passes into a zone 60 lower down where the blast has no effective force and where the matte is brought in contact with the coke which gives up its carbon to the sulfur and becomes sulfid of carbon which is a volatile product and passes up and 67 is burned or consumed in the smelting zone and converted into sulfurous acid which will again unite with any oxids present in the ore mixture, in the space above the smelting zone or where fusion takes place.

Iron may be carburized in the zone where the sulfur is removed instead of in high stacks or furnaces as is now done.

The slag is drawn off at the bottom of the zone where the sulfur is removed, and as copper sulfid is lighter and therefore on top of the gold, silver and lead when reduced to the metallic state, it may be drawn off below the slag as shown in the drawing. The lead, gold and silver passes lowest and is tapped out at 80 the bottom of the furnace.

All smelting processes require the mixture to contain sufficient silica to unite with all metals not wanted, to make a slag.

The accompanying drawing is a vertical 85 section of a furnace suitable for practicing my improved process. In this drawing the different zones are illustrated by shading. Let the numeral 5 designate the body of the furnace which is provided with a bustle pipe 90 6 from which air is supplied to the twyers 7 through conduits 8. These twyers deliver air to the central part of the fusion or smelting zone the depth and location of which is indicated by the two dotted horizontal lines A 95 and B which are exteriorly located in order to better define the said zone. Below the line B and between the lines B and C, the zone for separating the sulfur from the matte is located. At the bottom of the 100 zone B C, is a shallow zone C D, where the slag is drawn off through an opening M communicating with a discharge spout F. Below the slag zone C D, is the copper matte zone D E, the copper matte being drawn off 105 through an opening G leading to a spout H; while in the bottom of the furnace is a zone I in which the gold, silver and lead accumulate, the same being drawn off through an opening J leading to a spout K. All of 110 these draw-off openings are normally closed by plugs L.

In practicing the process the fuel as well as the ores to be treated are discharged into the furnace through an opening 9 normally closed by a gate 10. In this view the ore 5 located above the fusion zone is designated by the numeral 12. This ore becomes molten in the zone A B where the blast is introduced through the twy whole 7. In this fusion or smelting zone, the matte is formed being 10 composed of the entire ore mass containing the sulfur, it being assumed that the ore is sulfid in character. This matte passes downwardly from the zone A B into the zone B C where it comes in contact with the coke of 15 the fuel, the carbon of which unites with the sulfur to form sulfid of carbon which is volatile and passes upwardly being burned or consumed in the fusion or smelting zone A B. It must be understood that the zone 20 B C is entirely below the air plane or the level which is reached by the air or blast from the twy whole. Hence in this zone the coke being removed from contact with the air is prevented from burning in the absence 25 of air to support combustion. As soon as the carbon is separated from the matte, in the manner heretofore explained, the slag is drawn off from the zone C D immediately 30 below the separating zone B C, through an opening E leading to the discharge spout F.

Below the slag zone C D, is the copper matte zone D E since the copper matte being heavier than the slag is lighter than the gold, silver and lead. The copper matte is drawn off from the zone D E through the opening 35 G communicating with the discharge spout F and finally the gold and silver together with the lead are drawn off from the zone I at the bottom of the furnace through the opening J communicating with the discharge 40 spout K.

Having thus described my invention, what I claim is:

The herein described sulfid ore smelting process consisting in the separation of the 45 sulfur from the fused ores in the space or zone of the furnace below the fusion zone, by bringing the ore matte in contact with the carbon of the coke, out of contact with the air blast, whereby the sulfur is removed 50 in the form of sulfid of carbon, leaving the lead, gold and silver in the metallic state and the copper as matte, substantially as described.

In testimony whereof I affix my signature 55 in presence of two witnesses.

JAMES H. BOYD.

Witnesses:

A. J. O'BRIEN,  
DENA NELSON.